

# UNITED STATES PATENT OFFICE.

CHARLES J. KIRK, OF NEW CASTLE, PENNSYLVANIA.

## METHOD OF COATING METALLIC SURFACES.

936,637.

Specification of Letters Patent. Patented Oct. 12, 1909.

No Drawing.

Application filed May 28, 1908. Serial No. 435,546.

To all whom it may concern:

Be it known that I, CHARLES J. KIRK, of New Castle, in the county of Lawrence and State of Pennsylvania, have invented a 5 certain new and useful Improvement in Methods of Coating Metallic Surfaces, of which the following is a full, clear, and exact description.

My invention relates to an improvement 10 in producing a non-corrodible surface on metals and it consists in first amalgamating the metal to be protected with zinc flue-dust and then depositing a metal on the surface produced by the amalgamation of the zinc 15 flue dust.

Heretofore metals have been coated with zinc, tin, and other metals by passing the metal to be coated through a molten bath of the metal of which the coating is composed. 20 Metals have also been coated by depositing the zinc or other metal electrolytically and they have also been coated by what is known as the sherardizing process.

I will now describe my invention so that 25 others skilled in the art may employ the same.

In the practice of my invention I first sherardize the metal to be coated. This may be done by packing the metal to be 30 coated in what is known as zinc flue dust, which contains about ten per cent. of oxid of zinc, and then placing the metal and the zinc flue dust in a suitable muffle from which the air is excluded and then subjecting it to 35 heat for a sufficient length of time to cause an amalgamation of the zinc with the metal to be coated. The muffle is then allowed to cool and the sherardized metal is withdrawn. Or the flue dust may be mixed with water 40 or oils and powdered charcoal to form a liquid or semi-liquid mass of paint or compound which is then applied to the surface of the metal to be sherardized either by dipping the metal in a bath of the compound or 45 by painting the surface of the metal with the same. The metal so painted or coated is then placed in a muffle and subjected to heat the necessary length of time after which the muffle may be opened without danger of explosion and the metal is withdrawn and allowed to cool. I have discovered that this

sherardized surface forms a base upon which tin, zinc, or other metal may be deposited by passing the sherardized metal through a molten bath of the metal used to form the 55 coating, and owing to its peculiar qualities it causes an adhesion or amalgamation of the molten zinc, tin, or other metal far greater than would exist between the original surface of the metal and such coating, 60 so much so that a coating having new and characteristic properties is produced on the surface of the sherardized metal. The second step of my process therefore consists in dipping the sherardized metal in a molten 65 bath of zinc, tin, or other metal in the usual manner employed in galvanizing, tinning and coating metals in a molten bath. As the metal is withdrawn from the bath the excess of molten metal may be wiped off in the 70 usual manner. The metal when so removed from the bath is ready for use or it may be subjected to various polishing and finishing steps well known in the art.

The advantages of my invention are that 75 as by the sherardizing step an amalgamation of the zinc and the metal to be coated, takes place, so in the dipping step an amalgamation of the sherardized surface and the metal composing the molten bath takes place, producing a durable, amalgamated surface on 80 the metal to be protected.

Having thus described my invention, what I claim and desire to secure by Letters Patent is:

1. The method of protecting metal, consisting in sherardizing the metal to form a primary coating and then dipping the article so treated in a bath of molten metal capable of uniting with said primary coating.

2. The method of protecting metal, consisting in sherardizing the metal to form a primary coating and then forming thereon a second metallic coating capable of uniting with the primary coating.

In testimony whereof, I have hereunto set my hand.

CHARLES J. KIRK.

Witnesses:

M. ARTHUR KELLER,  
M. A. BARTH.